

July 15, 1930.

A. F. BEMIS

1,770,507

SYNTHETIC LUMBER

Filed Nov. 20, 1926

*Fig. 1*



*Fig. 2*



*Fig. 3*



*Inventor*  
Albert F. Bemis,  
by Robert Cushman Woodbury,  
Atty's.

## UNITED STATES PATENT OFFICE

ALBERT F. BEMIS, OF NEWTON, MASSACHUSETTS, ASSIGNOR TO BEMIS INDUSTRIES, INC., OF BOSTON, MASSACHUSETTS, A CORPORATION OF DELAWARE

## SYNTHETIC LUMBER

Application filed November 20, 1926. Serial No. 149,764.

This invention relates to an improved form of building material which may be conveniently termed synthetic lumber and may be provided either in sheets of any desired dimensions to form a substitute for lathes and plaster, sheathing, or ordinary wall board, or in thicker sections may be substituted for boards, brick work and various other building materials which are designed to form portions of walls, floors or roofs and are required to have a moderate degree of structural strength.

The invention more particularly pertains to the formation of composite lumber from sheets or laminations of fibrous material preferably fiber board and frangible plastic or cementitious material such as gypsum or the like. Heretofore it has been common in the art to provide thin fiber boards which have had certain inherent defects, such as a tendency to warp, inability to resist moisture, excessive expansion and contraction, only moderate compressive and tensile strength, rather poor nailing qualities and the like. It has also been usual to provide slabs of cementitious material, such as gypsum, with thin fibrous covering sheets of flexible material, such as paper or cardboard; slabs of this character having low tensile and bending strength, poor heat insulating qualities, comparatively poor nailing qualities and a tendency to break or crack easily, as well as being particularly difficult to ship and handle. Furthermore, this material is comparatively heavy in proportion to its heat insulating qualities and tensile or bending strength.

The present invention by combining the characteristics of the separate materials indicated above provides a building material which has the advantages common to both of the types of material previously used, with the disadvantages thereof reduced in degree or eliminated, thus being suited to a wide range of uses. The synthetic lumber disclosed herein, which comprises fiber boards located at either side of a frangible core, has comparatively good tensile and bending strength as well as a satisfactory degree of compressive strength and does not have an objectional tendency to swell or warp under conditions of high humidity. Preferably the fiber board is provided with a rough, irregular, or semi-villous surface whereby it may be firmly bound to the cementitious core and whereby the outer surface of the lumber may be adapted to receive plaster, stucco, etc. In proportion to its strength and moisture resistant qualities it is comparatively light and may provide very good heat insulation, while having better nailing qualities than either the conventional fiber board or the conventional gypsum slabs; and furthermore, it may be easily worked or shaped by ordinary carpenter's tools and may be handled, piled and shipped without requiring special care.

The above and further advantageous features of the invention will be apparent to those skilled in the art upon a reading of the subjoined description and claims in conjunction with the accompanying drawings in which

Fig. 1 is a perspective view of a portion of a sheet of the improved synthetic lumber;

Fig. 2 is a cross sectional view of the same; and

Fig. 3 is a similar view of a thicker piece of the material.

The composition lumber herein disclosed may be made of many suitable materials, but preferably includes outer layers of fiber board having considerable inherent stiffness or tensile strength, for instance, material formed of felted vegetable fibers such as wood fibers, or material, which is made from bagasse fibers which have been only partially cooked and therefore retain substantially all their original strength; these materials possessing numerous interstices or air cells so that their heat insulating qualities are comparatively high and having rough, somewhat villous surfaces to permit intimate bonding with cementitious material. Rather than material of this character a fiber board having the characteristics commonly associated with other ordinary fibrous wall boards may be used.

Between the fiber boards 1 of such a character, is poured or otherwise located plastic material 2, such as calcined gypsum, with or without suitable aggregate; preferably pressure is then applied to insure intimate bond-

ing of the fibers and the plastic material. For many purposes the thickness of the gypsum layer and of each of the fiber boards preferably may be substantially equal, but the thickness of the laminations may be somewhat varied in order to adapt the lumber to individual uses and installations. For example, in a case where heat insulation is particularly desired, the fiber board, insulite or celotex layers may be made thicker, while in other cases where moisture resistance is a prime requisite, the inner gypsum core may be somewhat thicker. The outer fiber board laminations and the gypsum core may be united by any suitable means, but preferably in such a manner that a rough fibrous surface of the board may firmly unite with the plastic material as it hardens, so that a strong union or bond is formed between the laminations of the lumber as designated by the numeral 3.

When it is desired to provide thick slabs or beams of this material, it will ordinarily be found advantageous to use several laminations of cementitious material and of fiber board in the manner illustrated in Fig. 3 rather than using thicker layers of fiber and gypsum.

Composite lumber of this type, which combines the separate advantages of the materials found therein, will be found adapted to a much wider variety of purposes. In its preferred embodiment when manufactured of materials such as referred to above, the outer layers will provide convenient means for applying stucco, plaster, or the like, due to the rough, fibrous surface which is a natural characteristic of this type of fiber board; obviously, however, the lumber may be provided with a finished surface in any conventional manner, and in certain cases a gypsum slab may form an outer layer of the lumber. The lumber may be readily handled and shaped, possesses greater structural strength and better nailing qualities than its component materials, and furthermore it provides satisfactory heat insulation, does not tend to expand, swell, or warp appreciably when exposed to high humidity or a high temperature and is comparatively fire resistant, while it possesses the ability to absorb rather than reflect sound waves.

I claim:

1. A sheet of wall board comprising outer layers of form retaining fiber board and an intermediate frangible layer of cementitious material which is bound by its inherent adhesive nature to the fiber board.

2. A sheet of wall board comprising outer layers of form retaining fiber board and an intermediate frangible layer, said fiber board having a roughened outer surface suitable for holding plaster or stucco.

3. A sheet of wall board comprising outer layers of form retaining fiber board and an

intermediate frangible layer, said fiber board providing heat-insulating layers.

4. Synthetic lumber comprising alternate layers of stiff, substantially form-retaining fiber board and of cementitious material, said fiber board having rough surfaces bonded to the cementitious material, the outer faces of said lumber being formed by the fiber boards whereby the cementitious material is protected against breaking.

5. A sheet of artificial lumber having relatively thick, light, form-retaining layers of cellular fibrous material having numerous interstices, and an inner layer of cementitious material, said outer layers constituting cushioning and stiffening means for the cementitious layer, and providing a board having good nailing qualities.

6. A sheet of artificial lumber having light, form-retaining outer layers of cellular fibrous material having numerous interstices, and an inner layer of cementitious material, said outer layers constituting cushioning and stiffening means for the cementitious layer, and providing a board having good nailing qualities, said outer layers being at least of approximately the thickness of said cementitious layer.

7. A sheet of artificial lumber having light, form-retaining outer layers of cellular fibrous material having numerous interstices, and an inner layer of cementitious material, said outer layers constituting cushioning and stiffening means for the cementitious layer, and providing a board having good nailing qualities, said outer layers being of substantially the thickness of the inner cementitious layer.

Signed by me at Boston, Massachusetts, this fourth day of November, 1926.

ALBERT F. BEMIS.

110

115

120

125

130